

## UNITED STATES PATENT OFFICE

2,376,867

## MANGANESE ALLOYS

Reginald S. Dean, Salt Lake City, Utah, assignor  
to Chicago Development Company, Chicago,  
Ill., a corporation of Illinois

No Drawing. Application July 12, 1941,  
Serial No. 402,239

9 Claims. (Cl. 148—12)

My invention relates to the preparation and heat treatment of alloys consisting essentially of manganese, iron and chromium, wherein the chromium content is in excess of the manganese content, and is particularly concerned with the preparation of such alloys which are highly resistant to atmospheric corrosion, possess the ability to withstand great extension by cold work without the hardening which is characteristic of austenitic stainless steels and irons heretofore known in the art, and, in addition, have the property of being hardened, without embrittlement, by heat treatment.

Alloys of manganese, chromium and iron, in which the chromium content exceeds the manganese content, have heretofore been suggested but, in all cases, those alloys whose properties have been investigated have contained a substantial content of carbon, of the order of 1% or more, although suggestions have been made for alloys where the carbon content was allegedly zero. There has, however, been no suggestion in the prior art of the amenability of such alloys to said heat treatments nor of the usual characteristics which are brought about by the heat treatments which are set out hereinafter in detail. Other alloys have been suggested in the prior art which contain manganese, chromium and iron, both carbon and silicon being present and the silicon comprising in excess of 3% and up to 8%.

The alloys of my invention are sharply distinguishable from those of the prior art in composition as well as in physical characteristics and properties. Thus, for example, the alloys of my invention must be substantially entirely free from the oxides of silicon and aluminum, carbon is substantially, and preferably entirely, absent, and silicon should not exceed 1% and is preferably present in amounts less than 0.7% and particularly close to 0%.

Again, there is a very definite and radical difference between the heat treatment proposed by the prior art as applied to alloys of manganese, chromium and iron and the heat treatments which I utilize. The heat treatment of the alloys of the present invention usually consists of a cooling, particularly quenching in water, cold working and reheating procedure, the cooling or quenching, as the case may be, taking place from a temperature preferably higher than 1100 degrees C. and particularly about 1200 degrees C. or not substantially less than 1200 degrees C. The heat treatment described in the prior art with respect to manganese, iron and chromium alloys involves heating the cast alloy to 1000 degrees

5 C. to 1100 degrees C. for several hours and then cooling in the furnace. Such a heat treatment does not produce increased strength in the alloys of my invention. Either it has no substantial effect on the hardness or produces a softening, depending upon the rate at which the alloys were cooled in casting.

It will be seen, therefore, as hereinafter pointed out in detail, that, by a suitable selection of alloy compositions and by heating of the alloys to approximately 1200 degrees C. and cooling or quenching, I may cold work the said alloys, by rolling, swaging or by any other means, to a very substantial extent without excessive hardening.

10 15 By excessive hardening, I refer to any hardness above about 25 as measured on the Rockwell C. scale. I have found that the range of alloy composition in which this phase of my invention may be practiced may be defined approximately as follows: From 7.5% to 22.5% manganese, from 15% to 32% chromium, the chromium content always exceeding the manganese content, and the balance being substantially all iron. A preferred range of the constituents of my alloys is 10 to 25 20% manganese, 24 to 30% chromium, balance iron.

As I have indicated hereinabove, when the alloys of my invention are heated to approximately 1200 degrees C. and slowly cooled they are rendered soft, the hardness of such alloys when heat treated in this way being from about zero to about 5 on the Rockwell C. scale. In this condition, I have found that these alloys may be cold worked to a very great degree without hardening above 25 as measured on the Rockwell C. scale. This ability to cold work to a great extent without undue hardening makes the alloys highly suitable for the production, among other things, of corrosion resistant thin sheets which have utility for various purposes as hereinafter pointed out.

40 45 It will be understood that by "slowly cooling" I mean the cooling of the alloy at a rate which would be obtained if it were allowed to cool in an ordinary heat-treating furnace, in general, by cooling at a rate such that at least six hours is required for the alloy to reach room temperature after the heat is turned off. It will be understood, of course, that the length of time required to bring the temperature of the heated alloy down to room temperature during the slow cooling process will depend, in part, upon the size and shape of the alloy element being treated. It 50 55 will also be understood that the slow cooling may

be carried out in air although, for best results, it should be carried out in an inert atmosphere.

I have also found that the alloys of my invention may effectively be placed in condition for extensive cold work by quenching them, preferably in water, from about 1200 degrees C. This treatment makes the alloys slightly harder than does the slow cooling process but renders them more susceptible to subsequent hardening by heat treatment.

Independently of which of the two methods described hereinabove is employed to treat the alloys prior to the cold working thereof, I have discovered that, by reheating the cold worked alloy to temperatures between about 400 degrees C. and 800 degrees C., substantial hardening takes place. In certain instances, this hardening may be brought to as high as Rockwell C. 59. In those of the alloys of my invention which contain not more than about 18% manganese, the alloys do not appear to become brittle by heating at any temperature within the aforementioned range. When the alloys contain 20% or upwards of manganese, embrittlement sometimes occurs by heating to temperatures of 550 degrees C. to 600 degrees C. Valuable hardness characteristics, however, may be developed in these latter alloys by utilizing lower hardening temperatures.

The following examples are illustrative of alloys falling within the scope of my present invention. It will be understood that various changes may be made therein, in the light of the guiding principles which I have disclosed, without in any manner departing from the spirit of my invention.

#### Example 1

High purity electrolytic iron, electrolytic chromium, and electrolytic manganese were melted together to produce a finished alloy containing 16% manganese, 25% chromium, balance iron. The alloy was heated to a temperature of 1200 degrees C. and quenched in water. The alloy was then reduced in area by swaging cold to the extent of 75%. In this condition, the hardness of the alloy was 25 on the Rockwell C scale. On heating to 600 degrees C., for two hours, the hardness of the alloy was Rockwell C. 53. On heating for a further period of two hours at 700 degrees C., the hardness was Rockwell C. 59. Even in this extremely hard condition, the alloy was remarkably tough.

#### Example 2

High purity electrolytic iron, electrolytic chromium and electrolytic manganese, were melted together to produce an alloy of 10% manganese, 30% chromium, balance iron. On heating said alloy to 1200 degrees C. and quenching and then reducing by cold work to the extent of 75% reduction in area, the hardness of the alloy was 18 on the Rockwell C scale. On reheating the quenched and cold worked alloy to a temperature of 600 degrees C. for two hours, the hardness increased to Rockwell C. 31. An additional two hours at 650 degrees C. increased the hardness to Rockwell C. 46 and a still further two hours at 700 degrees C. increased the hardness to Rockwell C. 53.

#### Example 3

High purity electrolytic iron, chromium and manganese were melted together to produce an alloy containing 19% manganese, 20% chromium, balance iron. Said alloy, when quenched from 1200 degrees C. and severely cold worked, had

a Rockwell C hardness of 21. On reheating for two hours at 600 degrees C., the hardness of the alloy became Rockwell C. 51. An additional heating of the alloy for two hours at 700 degrees C. increased the hardness to Rockwell C. 53.

#### Example 4

High purity electrolytic iron, chromium and manganese were melted together to produce an alloy containing 20% manganese, 24% chromium, balance iron. This alloy, when quenched from 1200 degrees C. and severely cold worked, had a Rockwell C hardness of 24. On reheating to a temperature of 550 degrees C., the alloy had a hardness of Rockwell C. 55.

In the practice of my invention, I prefer to employ electrolytic iron, electrolytic chromium and electrolytic manganese of high purity so as not to introduce deleterious constituents into the alloys. I have found, for example, that the presence of oxides of aluminum and silicon, such as are present in silico-thermic or alumino-thermic manganese or ferro-manganese prevents the effective practice of my invention. While the manganese which I employ may be produced by a vacuum distillation process, I prefer, particularly, to employ electrolytic manganese having a purity of at least about 99.0% and preferably of 99.9%.

By virtue of their hardening by reheating after quenching, particularly with intermediate cold work, my alloys are particularly useful for various purposes as, for example, gears, bearings, armour plate, and for purposes, in general, where case-hardened nickel or nickel-chromium steels have heretofore been used. The alloys of my present invention, hardened as described herein, have a wide utility in articles of cutlery, ball and roller bearings, tools and dies, especially saws, and other tools which are necessarily exposed to corrosive influences. In the soft state, the alloys of my present invention may be employed for cooking utensils and other purposes where a relatively soft material of satisfactory working qualities and a high degree of stainlessness is desired. They may also be utilized in the aircraft and automotive industries such as for the manufacture of thin sheets, of very high strength, for the fabrication of airplane wings or the like.

What I claim as new and desire to protect by Letters Patent of the United States is:

1. A process of producing stainless alloys of iron, chromium and manganese in the form of greatly cold worked rods, sheet or wire which comprises selecting an alloy within the composition range 7.5 to 22.5 per cent manganese, 15 to 32 per cent chromium, the chromium content always exceeding the manganese content, the balance being substantially all iron, heating said alloy to approximately 1200 degrees C., cooling, and subjecting the same to extensive cold work.

2. A process of producing stainless alloys of iron, chromium and manganese in a hardened but not brittle state and in a form obtained by a relatively large amount of cold work, which comprises selecting an alloy of iron, manganese and chromium within the composition range 7.5 to 22.5 per cent manganese, 15 to 32 per cent chromium, the percentage of chromium always exceeding that of the manganese, balance substantially all iron, heating said alloy to not substantially less than 1200 degrees C., cooling said alloy, extensively cold working said alloy, and then hardening by heating to a temperature between 400 degrees and 800 degrees C.

3. A process of producing stainless alloys of iron, chromium and manganese in a hardened but not brittle state and in a form obtained by a relatively large amount of cold work, which comprises selecting an alloy of iron, manganese and chromium within the composition range 7.5 to 18 per cent manganese, 16 to 30 per cent chromium, the chromium always exceeding the manganese, balance substantially all iron, heating said alloy to approximately 1200 degrees C., 10 quenching said alloy, extensively cold working said alloy, and then hardening by heating to temperatures between 400 degrees and 800 degrees C.

4. A process of producing thin sheets of stainless alloys of iron, chromium and manganese in a hardened state which comprises selecting an alloy from the composition range 10 to 20 per cent high purity manganese, 24 to 30 per cent high purity chromium, balance substantially all high purity iron, heating such alloy to approximately 1200 degrees C., cooling, cold rolling said alloy to the desired dimensions, and reheating said alloy to a temperature between 400 degrees C. and 800 degrees C.

5. Stainless alloys consisting essentially of manganese, chromium and iron, substantially entirely free of carbon and of oxides of aluminum and silicon, said alloys being in hardened form resulting from cooling from approximately 1200 degrees C., extensively cold working, and reheating between about 400 degrees C. and 800 degrees C., the alloy constituents being present in substantially the following proportions: 7.5 to 22.5 per cent of manganese, 15 to 32 per cent of chromium, the chromium content always exceeding that of the manganese, and balance substantially all iron.

6. Stainless alloys, in the form of thin sheets, consisting essentially of manganese, chromium and iron, substantially entirely free of carbon and 40

of oxides of aluminum and silicon, said alloys being in hardened form, resulting from cooling from approximately 1200 degrees C., rolling into sheet form, and reheating within the range of about 400 degrees C. to 800 degrees C., the alloy constituents being present in substantially the following proportions: 7.5 to 22.5 per cent of manganese, 15 to 32 per cent of chromium, the chromium content always exceeding that of the manganese, and balance substantially all iron.

5 7. A cold worked alloy consisting essentially of iron, chromium, and manganese, said alloy having a hardness of not more than 25 on the Rockwell C scale and resulting from heating said alloy to approximately 1200 degrees C. and cooling, said alloy containing from 7.5 to 22.5% manganese, from 16 to 30% chromium, balance substantially all iron, the chromium content being always in excess of the manganese content, said 15 alloy being substantially entirely free from carbon and oxides of silicon and aluminum.

20 8. A hardened alloy of iron, chromium and manganese, said alloy being made from high purity metals and containing from 7.5 to 22.5% manganese, from 16 to 32% chromium, the chromium content always exceeding the manganese content, balance substantially all iron, said alloy having been cooled from about 1200 degrees C., severely cold worked, and reheated to a temperature between 400 and 800 degrees C.

25 9. A hardened alloy of iron, chromium and manganese, said alloy being made from high purity metals and containing from 10 to 20% manganese, from 24 to 30% chromium, balance substantially all iron, the hardening of said alloy resulting from heating the same to approximately 1200 degrees C., quenching in water, and reheating to an elevated temperature.

REGINALD S. DEAN.